

May 3, 1938.

C. E. WOODDELL ET AL

2,115,897

ABRASIVE ARTICLE

Filed May 15, 1935

Fig. 1.



Fig. 2.



Fig. 3.



Fig. 4.



Fig. 5.



Fig. 6.



INVENTOR.

CHARLES E. WOODDELL  
CHARLES S. NELSON  
ROY LINCOLN

BY

*R. B. Binner*

ATTORNEY.

## UNITED STATES PATENT OFFICE

2,115,897

## ABRASIVE ARTICLE

Charles E. Wooddell and Charles S. Nelson, Niagara Falls, and Roy Lincoln, Buffalo, N. Y., assignors, by mesne assignments, to The Carborundum Company, Niagara Falls, N. Y., a corporation of Delaware

Application May 15, 1935, Serial No. 23,144

## 1 Claim. (Cl. 51—188)

This invention relates to improved abrasive articles. More specifically the invention is concerned with abrasive belts or bands adapted for rotation about pulleys or for mounting on wheels provided with a yieldable and resilient peripheral surface.

In copending application Serial No. 606,632, filed April 21, 1932, we have described and claimed abrasive articles of the class described wherein blocks of bonded abrasive material are attached to a flexible backing by a layer of resilient material of a character and thickness such that the device is adapted to yield locally under the pressures applied in grinding, rubber being the preferred cement for the purpose. In certain embodiments of that invention a layer of soft rubber is provided of sufficient thickness and resilience to permit the abrasive blocks to yield with respect to the backing material to which the soft rubber is attached.

We have now discovered that certain synthetic resins such as certain polyhydric alcohol-polybasic acid condensation products or certain modified vinyl resins have the requisite combination of properties to be suitable for use in place of the soft rubber disclosed in application Serial No. 606,632 and that articles cemented with these resins exhibit grinding characteristics not attainable with rubber cements.

Understanding of our invention will be assisted by reference to the accompanying drawing wherein:

Figure 1 is a top view of a portion of an abrasive belt or band employing one modification of our invention;

Figure 2 is a cross sectional view along the lines II—II of Figure 1;

Figure 3 is a top view of a portion of an abrasive belt or band embodying another modification of our invention;

Figure 4 is a sectional view along the lines IV—IV of Figure 3;

Figure 5 is a section of one form of a wheel embodying our invention; and

Figure 6 is a partial section of a modification of Figure 5.

Referring to the drawing, the belts or bands of Figures 1 to 4 comprise a backing 1 to which are attached blocks of bonded abrasive material 3 by a cement 2. In Figures 5 and 6 there is shown an embodiment of the invention wherein a band of the type illustrated in Figures 3 and 4 is mounted on a wheel comprising a rigid core 4 with a peripheral layer 5 of resilient and yieldable material such as soft rubber.

The backing 1 may be made of metal, fabric, leather or other suitable material but we prefer to employ a one piece jointless metal band such as a band of spun steel. The backing must be sufficiently flexible to permit the band to bend 5 and straighten out, as is required by a belt operating about pulleys or to yield slightly under the pressures applied in grinding when the band is mounted on a wheel having a periphery of resilient material as illustrated in Figures 5 and 6. 10 A spun steel band about .010-.015 inch in thickness has been found to be satisfactory.

The abrasive blocks 3, illustrated in Figures 1 and 2 as individually formed blocks, may be made in any of the usual ways. For example, they may 15 be bonded with a ceramic, resin, rubber, silicate or other desired bond in ways well-known to the art. Similarly, they may be prepared by any of the known methods such as by pressing, sheeting, tamping or the like, thus making it possible 20 to furnish abrasive bands or belts in which the abrasive portion has the characteristics desired. This adaptability of the invention to the use of various types of abrasive bodies is a valuable 25 feature of the invention as it permits furnishing abrasive belts having any desired grinding characteristics.

Where blocks are formed by fracturing a continuous body of bonded abrasive, such as are illustrated in Figures 3 and 4, the abrasive body may conveniently be formed as a continuous block of the required dimensions, cemented to the backing, and then fractured to permit bending of the belt. This method of making bands is particularly adapted for use on 30 backings which can be straightened out into a plane surface although it may be applied to circular bands by molding the abrasive as hollow cylinders of the required dimensions.

We have found that the choice of a cement 2 40 for attaching the abrasive bodies to the backing material is an important consideration in the preparation of satisfactory belts. As will appear from a consideration of the movement of a backing when it is used as a belt moving over two or 45 more pulleys, the cement is subjected to rather severe stresses due to the continued and repeated curving and straightening of the backing. Since the abrasive blocks are attached rigidly to the backing, flexure of the belt occurs between 50 the blocks but such flexure transmits stresses to the cement which tend to tear the block from the belt as the backing tends to assume a curvature equal to that of the pulleys. It is therefore desirable to provide the pulleys with a peripheral 55

layer of yieldable material such as soft rubber in order that the pulleys may absorb part of these stresses.

Because of these stresses the cement must be unusually strong and tough, highly adhesive to both the backing and the abrasive blocks, and resilient enough to absorb the stresses set up. A brittle cement, even though it has high tensile strength, is unsatisfactory because it cracks and allows the abrasive blocks to become detached.

The stresses imposed upon the cement are accentuated by the pressures applied through the work piece when the belt or band is in use.

We will now illustrate our invention with a number of specific examples, it being understood that the examples are for illustrative purposes only and are not intended to be limitative.

*Example 1*

20 Abrasive sticks  $2\frac{3}{8}$  inches long by  $\frac{3}{8}$  inch wide by  $\frac{1}{4}$  inch thick were made up with 80 grit fused alumina grain and 10% of a phenolic resin bond in the manner described and claimed in a patent to Harry C. Martin, No. 1,626,246. A  $2\frac{3}{8}$ " x  $\frac{3}{8}$ " 25 surface was coated with a rather thick solution in acetone of a modified vinyl resin having a softening point of about  $150^{\circ}$  C. and known as "Alvar V 15 H 70". This resin is prepared by hydrolyzing polyvinyl acetate and reacting the product with acetaldehyde as described in British Patent No. 351,082.

A steel band  $2\frac{3}{8}$ " wide,  $\frac{3}{16}$ " thick and 12 inches in diameter was mounted on a pulley, its outer surface was sandblasted, and a thinner solution 35 of the resin described above was applied to the sandblasted surface. The abrasive blocks were then mounted on the band with the cement-coated surfaces in contact with each other leaving  $\frac{1}{4}$ " 40 spaces between blocks, and a wet cloth was tightly tied around the assembly. Upon drying the wet cloth shrinks and tightens.

The assembled band was dried for 24 hours at room temperature and for 48 hours at  $120^{\circ}$  F. to remove the solvent. It was then mounted on an 45 expandible pulley provided with a peripheral layer of soft rubber, dressed with a silicon carbide brick and speeded to 2500 surface feet per minute. The band was used for grinding until the blocks had worn very thin without damage to the resin

cement or difficulty from the blocks becoming detached.

*Example 2*

A band was prepared in a manner similar to that described in Example 1 except that the cement used on the abrasive blocks consisted of a mixture of 100 parts of a flexible alkyd resin known to the trade as "1353 F Glyptal", 10 parts of pulverized cork and 2 parts of zinc oxide, while the band was painted with an acetone solution of the same alkyd resin. The cement applied to the blocks was melted and was free from solvent.

After assembling, this band was cured in an oven by raising the temperature of the oven to  $350^{\circ}$  F. in 5 hours and holding that temperature for 16 hours.

*Example 3*

A band was prepared as described in Example 2 except that ceramically bonded sticks of silicon carbide were used instead of the resin bonded fused alumina of Examples 1 and 2.

As was pointed out above, our invention has the advantage that it is adapted to use abrasive bodies of any desired composition. It has the 25 added advantage over the invention of our co-pending application that the resin cements provide a more rigid mounting than rubber and the wheels and belts of the present invention therefore provide a grinding action not obtainable by 30 a resiliently mounted block and yet one which is somewhat softer than can be obtained with the conventional rigidly bonded abrasive wheel.

Having described our invention and illustrated it with specific examples, we declare that what 35 we claim is:

An abrasive article comprising a flexible band, a plurality of blocks of bonded abrasive material attached to said band by a resin layer containing a major proportion of a synthetic resin, said layer being flexible enough to permit the band to bend between the blocks, and strong enough to retain the band flat against the blocks and to prevent the blocks from yielding locally under the pressure of grinding.

CHARLES E. WOODDELL.  
CHARLES S. NELSON.  
ROY LINCOLN.